

# UNITED STATES PATENT OFFICE.

UMATA OKAZAKI, OF KITAGUCHI, OKAYAMA-SHI, OKAYAMA-KEN, JAPAN, ASSIGNEE  
TO HARRY E. RIDINGS, OF YOKOHAMA, JAPAN.

## COMPOSITION OR PULP.

1,278,199

Specification of Letters Patent. Patented Sept. 10, 1918.

No Drawing.

Application filed November 1, 1917. Serial No. 199,797.

*To all whom it may concern:*

Be it known that I, UMATA OKAZAKI, a subject of Japan, residing at Kitaguchi, Okayama-Shi, Okayama-Ken, Japan, have invented a new and useful Composition or Pulp, of which the following is a specification.

The object of my invention is the production of a fibrous composition, or pulp, from which paper can be made, the chief constituent being leaves of sugar cane, which at the present time are not only not used in paper-pulp but are useless for any purpose and are wasted.

My composition consists of sugar-cane leaves, treated with water, caustic soda, lime, chlorid of lime, and sulfuric acid.

In preparing the composition the leaves are chopped into pieces and cleaned by air, then boiled with caustic soda and lime for about four hours; to 100 parts of leaves are used .6 parts of caustic soda and .5 (one-half) part of lime. Then it is washed in a sieve-like vat, and beaten and washed in

a beating machine. The fibers having been separated in the beating machine, are bleached by a solution of chlorid of lime and sulfuric acid, using to each 100 parts of the fibrous substance 6.5 parts of chlorid of lime, .5 (one-half) part of sulfuric acid, and water as required; the fiber remains in this solution about four hours during which time it is steamed with steam at 75 to 80 degrees centigrade; this steaming shortens the bleaching process much. The bleached fiber is rinsed with clear water in an oscillating strainer, passing from which it is sized and made ready to go into the millboard machine. Then after going through a drying machine, it comes out finished pulp ready to be made into paper.

I claim:

A fibrous composition, or pulp, from which paper can be made, consisting of sugar-cane leaves, treated with water, caustic soda, lime, chlorid of lime, and sulfuric acid, or any similar chemicals.

UMATA OKAZAKI. [L. S.]